

Jan. 18, 1938.

J. C. MORRELL

2,105,549

CONVERSION OF HYDROCARBON OILS

Filed Dec. 20, 1934



## UNITED STATES PATENT OFFICE

2,105,549

## CONVERSION OF HYDROCARBON OILS

Jacque C. Morrell, Chicago, Ill., assignor to Universal Oil Products Company, Chicago, Ill., a corporation of Delaware

Application December 20, 1934, Serial No. 758,443

7 Claims. (Cl. 196—48)

This invention particularly refers to an improved process for the treatment of hydrocarbon oils of relatively wide boiling range embodying the cooperative steps of topping, cracking, coking and reforming.

In one specific embodiment, the invention comprises subjecting charging stock for the process, comprising an oil of relatively wide boiling range, such as crude petroleum, for example, to fractional distillation whereby it is separated into relatively low-boiling and high-boiling fractions, subjecting said low-boiling fractions of the charging stock, including its components within the boiling range of motor fuel as well as, when desired, somewhat higher boiling fractions such as naphtha, kerosene or kerosene distillate and the like, to conversion or reforming in a heating coil, partially cooling the resulting products by indirect heat exchange with hydrocarbon oil charging stock for the process, whereby to retard or arrest their conversion, heat the charging stock for the purpose of effecting or assisting said fractional distillation thereof and remove heavy polymers and residual liquids from the vaporous conversion products, subjecting the vaporous conversion products to fractionation whereby their insufficiently converted components are condensed as reflux condensate and separated into selected relatively low-boiling and high-boiling fractions, subjecting fractionated vapors of the desired end-boiling point to condensation, recovering and separating the resulting distillate and gas, subjecting high-boiling fractions of said reflux condensate to conversion conditions of elevated temperature and superatmospheric pressure in a separate heating coil, introducing the resulting heated products into a coking chamber wherein the residual liquid conversion products are reduced to substantially dry coke, subjecting low-boiling fractions of said reflux condensate to independently controlled conversion conditions of elevated temperature and superatmospheric pressure in another separate heating coil, introducing the resulting highly heated products into said coking chamber, withdrawing the vaporous products from the coking chamber and separating therefrom tars and similar high coke-forming materials, returning the latter to the coking chamber and subjecting the remaining vaporous products from the coking operation to further conversion in the first mentioned heating coil together with said low-boiling fractions of the charging stock. The high-boiling fractions of the charging stock may be supplied direct to the coking chamber or subjected to conversion

together with the high-boiling fractions of the reflux condensate or, when desired, both the high-boiling fractions of the reflux condensate and the high-boiling fractions of the charging stock may be supplied direct to the coking chamber without passing through said separate heating coil.

It will be apparent from the foregoing as well as from the following further description of the process of the present invention that its various features and the various stages of the process are interdependent and mutually contribute to produce the desired final results.

The accompanying diagrammatic drawing illustrates one specific form of apparatus in which the process of the invention may be accomplished.

Referring to the drawing, hydrocarbon oil charging stock preferably comprising, as already mentioned, an oil of relatively wide boiling range such as crude petroleum or the like, preferably containing a substantial proportion of both relatively low-boiling and relatively high-boiling fractions, is supplied through line 1 and valve 2 to pump 3 by means of which it is fed through lines 4 and 5 and valve 6 into heat exchanger 7 wherein it is subjected to indirect heat exchange with hot conversion products of the process and thereby heated to a temperature sufficient to effect its substantial vaporization and fractional distillation. The heated charging stock is discharged from the heat exchanger through line 8 and valve 9 into distilling and fractionating column 10. The charging stock may, of course, be subjected to heating in any well known manner, not illustrated, instead of or in conjunction with the heating accomplished in heat exchanger 7.

Distilling and fractionating column 10 may be operated at any desired pressure ranging from substantially atmospheric to a high superatmospheric pressure of the order of several hundred pounds per square inch but preferably a superatmospheric pressure is employed in this zone sufficient to permit the passage of the overhead vaporous products from column 10 to and through heating coil 21 without the aid of a vapor pump or compressor. The charging stock is separated by fractional distillation in column 10 into selected relatively low-boiling and high-boiling fractions. The latter are collected as bottoms in the lower portion of column 10 from which they are withdrawn through line 11 and valve 12 to pump 13, by means of which they are fed through line 14 and may be directed through line 15, valve 16 and line 43 to conversion in heating coil 55

45, or this material may be directed through valve 17 in line 14 through lines 70, 58 and 47 into coking chamber 49. The selective low-boiling fractions of the charging stock are withdrawn as 5 fractionated vapors from the upper portion of column 10 through line 18 and valve 19 and is directed through line 20 to heating coil 21. It is, of course, within the scope of the invention, when desired, to employ a suitable vapor pump or compressor in line 18 in case heating coil 21 is operated at a higher pressure than that employed in column 10 or, when desired, the fractionated vapors may be subjected to condensation and the resulting distillate supplied by means of a suitable pump to heating coil 21, although these alternative methods of operation are not illustrated in the drawing.

Heating coil 21 is located within a furnace 22 of any suitable form by means of which the oil passing through the heating coil is subjected to the desired relatively high conversion temperature at any desired pressure. The hot conversion products are discharged from heating coil 21 through line 23 and valve 24 into heat exchanger 7 wherein they are cooled sufficiently, by indirect contact with charging stock for the process, supplied to this zone as previously described, to prevent any appreciable further conversion thereof. Partial cooling of the conversion products in heat exchanger 7 serves to remove therefrom by condensation undesirable heavy liquid components such as heavy polymers, residual liquid and the like which may be withdrawn from the heat exchanger 35 and directed through lines 25 and 77 and valve 26 to column 10 wherein they commingle with the high-boiling fractions of the charging stock and are directed therewith to further treatment as will be later more fully described. As an alternative method of operation the condensate from heat exchanger 7 may, when desired, be directed through valve 78 in line 25 to pump 79 by means of which it is supplied through line 80, valve 81 and line 58 to coking chamber 49. The vaporous conversion products remaining uncondensed in heat exchanger 7 are directed therefrom through line 27 and valve 28 to fractionation in fractionator 29.

The components of the vaporous conversion products supplied to fractionator 29 boiling above the range of the desired final light distillate product of the process are condensed in this zone as reflux condensate and the reflux condensate is separated by fractional distillation into selected 55 relatively low-boiling and high-boiling fractions which are subjected to selective conversion, as will be later more fully described.

Fractionated vapors of the desired end-boiling point are withdrawn, together with uncondensable gas produced within the system, from the upper portion of fractionator 29 through line 30 and valve 31 and are subjected to condensation and cooling in condenser 32. The resulting distillate and gas passes through line 33 and valve 60 65 34 to collection and separation in receiver 35. Uncondensable gas may be released from the receiver through line 36 and valve 37. Distillate may be withdrawn from receiver 35 through line 38 and valve 39 to storage or to any desired further treatment. A regulated portion of the distillate collected in receiver 35 may, when desired, be recirculated by well known means, not shown in the drawing, to the upper portion of fractionator 29 to serve as a cooling and re-

fluxing medium in this zone for assisting fractionation of the vapors and to maintain the desired vapor outlet temperature from the fractionator.

The high-boiling fractions of the reflux condensate formed in fractionator 29 are withdrawn from the lower portion of this zone through line 40 and valve 41 to pump 42, by means of which they are fed through line 43 and valve 44 and may be directed through valve 74 and supplied, either alone or together with the high-boiling oils from the lower portion of column 10, which may be directed into line 43 in the manner previously described, to conversion in heating coil 45 or the high-boiling fractions of the reflux condensate may be diverted from line 43 through line 75 into line 70 to be supplied therefrom, together with the heavy liquids from separator 65 and also, when desired, together with the bottoms from column 10 through line 58 and line 20 47 into coking chamber 49.

The oil supplied to heating coil 45 is subjected to the desired conversion temperature by means of heat supplied from a furnace 46 of any suitable form and the stream of hot conversion products is discharged from the heating coil through line 47 and valve 48 into coking chamber 49. Heating coil 45 may, of course, be eliminated, when desired, by supplying both the bottoms from distilling and fractionating column 10 and the high-boiling fractions of the reflux condensate from fractionator 29 direct to coking chamber 49 in the manner previously described, in which case the heat required to effect conversion and coking of these relatively high-boiling oils in coking chamber 49 is derived from the highly heated conversion products supplied to this zone from heating coil 55, as will be later more fully described.

Selected relatively low-boiling fractions of the reflux condensate formed in fractionator 29 may be withdrawn from any suitable intermediate point or plurality of points in this zone and, in the case here illustrated, this material is directed through line 50 and valve 51 to pump 52 by means of which it is fed through line 53 and valve 54 to conversion in heating coil 55, wherein it is heated to the desired conversion temperature, preferably at a substantial superatmospheric pressure, by means of heat supplied from a furnace 56 of any suitable form. The stream of hot conversion products is discharged from heating coil 55 through line 57 and may be directed through line 58, valve 59 and line 47 into coking chamber 49, together with the stream of hot conversion products from heating coil 45, or the conversion products from heating coil 55 may be separately introduced into the coking chamber at any desired point or plurality of points in this zone. Provision is shown in the drawing for directing all or a portion of the hot conversion products from heating coil 55 through valve 60 in line 57 into the lower portion of the coking chamber, wherein they commingle with and serve to supply additional heat to the materials undergoing coking in this zone.

Coking chamber 49 may be operated at any desired pressure ranging from substantially atmospheric to several hundred pounds per square inch superatmospheric and preferably a superatmospheric pressure is employed in this zone sufficient to permit the passage of vapors products therefrom through heating coil 21 without the use of a vapor pump or compressor. The liq-

uid components of the conversion products supplied to the coking chamber are subjected to further distillation and/or conversion in the zone and the resulting residue is reduced to substantially dry coke. The coke may be allowed to accumulate within the coking chamber until it is substantially filled, following which the chamber may be isolated from the rest of the system, cleaned and prepared for further operation. When desired, a plurality of coking chambers may be employed, although only one is illustrated in the drawing, in which case they preferably are alternately operated, cleaned and prepared for further operation so that the duration of the operating cycle of the process is not limited by the capacity of the coking zone. Chamber 49 is provided with a suitable drain-line 61 controlled by valve 62 which may also serve as a means of introducing steam, water or any other suitable cooling medium into the chamber, after its operation is completed and after it has been isolated from the rest of the system, in order to hasten cooling and facilitate the removal of coke from the chamber.

Vaporous products are withdrawn from the upper portion of the coking chamber through line 63 and valve 64 to separator 65, wherein any heavy components or entrained liquid particles such as tars and similar heavy liquids of a high coke-forming nature are removed from the vapors. When desired, in order to assist the removal of said high-boiling materials from the vaporous products from the coking zone, a regulated portion of the charging stock may be directed from pump 3 through valve 66 in line 4 into separator 65 and, when desired, regulated portions of either the low-boiling or high-boiling fractions of the reflux condensate formed in fractionator 29 may be supplied, by well known means, not shown in the drawing, to separator 65 for the same purpose. The high coke-forming liquids separated from the vaporous products from the coking chamber in separator 65 are withdrawn from the lower portion thereof through line 67 and valve 68 to pump 69 by means of which they are returned through means of line 10, valve 71, line 58 and line 47 to coking chamber 49 for further treatment and reduction to coke.

The vaporous products from the coking chamber escaping condensation in separator 65 are directed therefrom through line 12, valve 73 and line 20 to further conversion in heating coil 21, together with the low-boiling fractions of the charging stock from column 10. It is, of course, within the scope of the invention, although not illustrated, to subject the vapors from separator 65 to condensation and to supply the resulting distillate by pump to conversion in heating coil 21, although this involves a considerable loss of heat by condensation of the vapor and is not the preferred method of operation.

The preferred range of operating conditions which may be employed in a process such as illustrated and above described may be approximately as follows: When a heating coil is employed for conversion of the heavy oils, comprising the high-boiling fractions of the charging stock or the high-boiling fractions of the reflux condensate or both, a conversion temperature ranging, for example, from 800 to 950° F. may be employed at the outlet from this zone, preferably with a superatmospheric pressure at this point in the system of from 100 to 500 pounds, or more, per square inch. The heating coil to which the relatively low-boiling fractions of the reflux condensate are supplied may utilize an outlet conversion temperature ranging, for example, from 900 to 1000° F. preferably with a superatmospheric pressure, measured at the outlet from this zone, of from 200 to 800 pounds, or more, per square inch. The coking chamber may employ any desired pressure ranging from substantially the same as that employed at the outlet from the preceding heating coil employing the lowest pressure down to substantially atmospheric pressure, although a superatmospheric pressure at least slightly above the pressure employed in the succeeding heating coil is preferred in this zone. The distilling and fractionating column wherein the charging stock is subjected to fractional distillation may employ any desired pressure ranging from substantially atmospheric to 500 pounds, or more, per square inch, superatmospheric pressure and preferably a superatmospheric pressure is employed in this zone slightly higher than that employed in the succeeding heating coil. The heating coil to which low-boiling fractions of the charging stock and the vaporous products from the coking chamber are supplied may utilize an outlet conversion temperature ranging, for example, from 950 to 1100° F. with any desired pressure ranging from substantially atmospheric to 500 pounds, or more, per square inch, the higher temperatures normally being employed when lower pressures are utilized. The fractionating, condensing and collecting portions of the system may employ pressures substantially the same or lower than that employed at the outlet from the last mentioned heating coil.

As a specific example of the operation of the process of the present invention as it may be accomplished in an apparatus such as illustrated and above described, the charging stock comprises a California crude of about 32.8° A. P. I. gravity containing approximately 5 per cent of material boiling up to 200° F. and approximately 36 per cent at 437° F. and this material is subjected to fractional distillation by means of heat supplied thereto by indirect heat exchange with the hot conversion products from the heating coil to which the low-boiling fractions of the charging stock are supplied. The charging stock is separated by said fractional distillation into fractions boiling above and below approximately 550° F. The fractional distilling stage of the system is operated at a superatmospheric pressure of approximately 200 pounds per square inch. Approximately 50 per cent of the charging stock, comprising its fractions boiling above approximately 550° F. are subjected, together with high-boiling reflux condensate from the fractionator of the cracking system, to a conversion temperature, measured at the outlet from the separate heating coil to which these materials are supplied, of approximately 920° F. at a superatmospheric pressure of approximately 200 pounds per square inch which pressure is substantially equalized in the succeeding coking chamber. Selected low-boiling fractions of the reflux condensate, having a boiling range of approximately 400 to 600° F., are subjected to another separate heating coil to an outlet conversion temperature of approximately 970° F. at a superatmospheric pressure of approximately 400 pounds per square inch and the highly heated products from this heating coil are introduced into the coking chamber. Tars and similar high-boiling materials separated from the vaporous products from the coking chamber are returned to the coking chamber. The re-

maining vapors, together with the low-boiling fractions of the charging stock, are subjected in the heating coil to which they are supplied to an outlet conversion temperature of approximately 5 1000° F. and the pressure utilized in this zone is substantially equalized with that in the distilling and fractionating column and the coking chamber. The stream of heated products from the last mentioned heating coil is cooled by indirect 10 heat exchange with the charging stock and by pressure reduction to a temperature of approximately 750° F. and the resulting partially cooled vaporous products are supplied to the fractionator of the system which is operated at a 15 superatmospheric pressure of approximately 50 pounds per square inch. This operation may produce, per barrel of charging stock, approximately 68 per cent of 400° F. end-point motor fuel having an octane number of approximately 20 75 by the motor method, the additional products of the process being approximately 50 pounds of relatively dry coke and the remainder uncon- densable gas.

I claim as my invention:

- 23 1. A process which comprises topping crude petroleum, thereby forming topped crude and a distillate containing natural gasoline fractions of the crude, distilling the topped crude to coke in a coking zone, combining vapors from the coking zone with said distillate, heating the resultant mixture in a heating coil sufficiently to enhance the anti-knock value of said gasoline fractions, fractionating resultant cracked vapors independently of said vapors from the coking zone and 35 separating relatively heavy and light reflux condensates therefrom, supplying such heavier reflux condensate to the coking zone for reduction to coke together with the topped crude, subjecting the lighter reflux condensate to independently 40 controlled cracking conditions of temperature and pressure in a second heating coil, and introducing resultant heated products into the coking zone to assist the coking of the topped crude and heavier reflux condensate therein.
- 45 2. The process as defined in claim 1 further characterized in that the topped crude and heavier reflux condensate, prior to introduction to the coking zone, are passed in admixture through a third heating coil and heated therein to a lower 50 conversion temperature than is maintained in the first-named and said second coils.
- 55 3. A process which comprises topping crude petroleum, thereby forming topped crude and a distillate containing natural gasoline fractions of the crude, distilling the topped crude to coke in a coking zone, separating relatively heavy fractions of the resultant vapors and returning the same to the coking operation, combining the remaining vapors from the coking zone with said 60 distillate, heating the resultant mixture in a heating coil sufficiently to enhance the anti-knock value of said gasoline fractions, fractionating resultant cracked vapors independently of said vapors from the coking zone and separating relatively heavy and light reflux condensates therefrom, supplying such heavier reflux condensate to the coking zone for reduction to coke together with the topped crude, subjecting the lighter reflux condensate to independently controlled 65 cracking conditions of temperature and pressure 70 cracking conditions of temperature and pressure

in a second heating coil, and introducing resultant heated products into the coking zone to assist the coking of the topped crude and heavier reflux condensate therein.

4. A process which comprises topping crude petroleum, thereby forming topped crude and a distillate containing natural gasoline fractions of the crude, distilling the topped crude to coke in a coking zone, combining vapors from the coking zone with said distillate, heating the resultant mixture in a heating coil sufficiently to enhance the anti-knock value of said gasoline fractions, fractionating resultant cracked vapors independently of said vapors from the coking zone and separating relatively heavy and light reflux condensates therefrom, heating such heavier reflux condensate to cracking temperature in a second heating coil and the lighter reflux condensate to higher cracking temperature in a third heating coil, and discharging heated products from said second and third coils into the coking zone and into contact with the topped crude undergoing coking therein.

5. The process as defined in claim 1 further characterized in that said distillate is supplied to the first-named coil directly and without prior condensation from the topping operation.

6. A process for producing anti-knock motor fuel from crude petroleum containing straight-run gasoline, which comprises topping the crude in a topping zone to vaporize the gasoline therefrom, removing topped crude from said zone and distilling the same to coke in a coking zone, combining vapors from the coking zone with the gasoline-containing vapors from the topping zone, 35 heating the resultant vaporous mixture in a heating zone sufficiently to increase the anti-knock value of the gasoline contained therein, fractionating resultant cracked vapors and subjecting resultant reflux condensate to independently controlled cracking conditions of temperature and pressure in a second heating zone, discharging the heated products from said second heating zone into the coking zone to assist the coking of the topped crude therein, and finally condensing the 40 fractionated vapors.

7. A process for producing anti-knock motor fuel from crude petroleum containing straight-run gasoline, which comprises topping the crude in a topping zone to vaporize the gasoline therefrom, removing topped crude from said zone and distilling the same to coke in a coking zone, combining vapors from the coking zone with the gasoline-containing vapors from the topping zone, heating the resultant vaporous mixture in a heating zone sufficiently to increase the anti-knock value of the gasoline contained therein, fractionating the resultant cracked vapors to separate relatively heavy and light reflux condensates therefrom, supplying such heavier reflux condensate to the coking zone for reduction to coke therein, subjecting the lighter reflux condensate to independently controlled cracking conditions of temperature and pressure in a second heating zone, discharging the heated products from said 65 second heating zone into the coking zone to assist the coking of the topped crude therein, and finally condensing the fractionated vapors.